

[54] COMPOSITE PROPELLANT CONTAINING  
POLYTETRAFLUOROETHYLENE POWDER  
AND BUTYL OR ETHYLENE-PROPYLENE  
RUBBER

[75] Inventors: Martin H. Kaufman; Edward M. Roy, both of China Lake, Calif.

[73] Assignee: The United States of America as represented by the Secretary of the Navy, Washington, D.C.

[22] Filed: Oct. 30, 1970

[21] Appl. No.: 90,210

[52] U.S. Cl..... 149/19.3, 149/19.91, 149/20,  
149/44, 149/76

[51] Int. Cl..... C06d 5/06

[58] Field of Search .... 149/19, 76, 44, 19.3, 19.91,  
149/20

[56] References Cited

UNITED STATES PATENTS

|           |        |                    |          |
|-----------|--------|--------------------|----------|
| 3,257,802 | 6/1966 | Kaufman.....       | 149/2 X  |
| 3,377,955 | 4/1968 | Hodgson .....      | 149/19 X |
| 3,395,055 | 7/1968 | Sparks et al. .... | 149/19 X |

|           |         |                    |          |
|-----------|---------|--------------------|----------|
| 3,476,622 | 11/1969 | Harada et al. .... | 149/19   |
| 3,513,043 | 5/1970  | Burnside .....     | 149/87 X |
| 3,577,289 | 5/1971  | Morrell .....      | 149/19   |
| 3,586,552 | 6/1971  | Potts et al. ....  | 149/19   |

Primary Examiner—Benjamin R. Padgett

Assistant Examiner—E. A. Miller

Attorney, Agent, or Firm—R. S. Sciascia; Roy Miller; Lloyd E. K. Pohl

[57] ABSTRACT

A process for the preparation of propellant molding powders having good ingredient quality control and good composition homogeneity comprising Teflon powder, butyl or ethylene-propylene rubber binder and an inorganic oxidizer. Metal fuels such as aluminum were also included, as were burning rate modifiers. The process comprises forming a homogeneous binder solution, adding the propellant ingredients and mixing to form a paste, extruding the paste through small cross-sectional orifices, blowing warm air or inert gas around the strands extruded from the orifices and collecting the strands by appropriate means.

7 Claims, No Drawings

**COMPOSITE PROPELLANT CONTAINING  
POLYTETRAFLUOROETHYLENE POWDER AND  
BUTYL OR ETHYLENE-PROPYLENE RUBBER**

**STATEMENT OF GOVERNMENT INTEREST**

The invention described herein may be manufactured and used by or for the Government of the United States of America for governmental purposes without the payment of any royalties thereon or therefor.

**BACKGROUND OF THE INVENTION**

The present invention relates to improved homogeneous propellant molding powder and to the process for preparation thereof.

For some time in the propellant field work has been directed toward devising and providing a versatile family of propellants to meet the future needs of the rocket system developers. The hydrocarbon-rubber binder systems now in use are highly unsaturated and are the major cause of chemical instability of the propellant grain. Chemical stability is important since chemical changes that affect the performance may occur during storage in uncontrolled environments. Moreover, the techniques by which they are used may introduce various process variables which prevent ballistic reproducibility. The present invention is for propellant powders which are highly homogeneous. The process eliminates a quality control problem, enhances reliability in regard to those features which are affected by homogeneity, and eliminates a potential safety hazard caused by free oxidizer.

**DESCRIPTION OF THE INVENTION**

In accordance with the present invention from about 50 to 70 percent by weight inorganic oxidizer and 10 to 20 percent by weight metal fuel were incorporated into a matrix comprising from about 2 to 10 percent by weight polytetrafluoroethylene (Teflon) and from about 5 to 10 percent by weight butyl or ethylene propylene rubber to form a paste. The paste was extruded through small cross-sectional area orifices producing strands of the formulation around which a high volume of warm air or inert gas was circulated by blowing means and the strands collected on conveyor belts or other means, followed by complete drying or curing under ambient conditions.

The matrix is prepared by mixing the selected rubber, butyl and/or ethylene-propylene, in a solvent such as petroleum ether which is preferred. However, hexane works satisfactorily with the ethylene-propylene rub-

bers. Butyl rubber is highly impermeable (a very desirable feature) and holds tenaciously to the solvent.

Propellant strands prepared by this process are highly homogeneous. The strands show no oxidizer on the surface and no material is segregated. Nothing is selectively lost by adherence to the mixing kettle, as often occurs in the well known shock-precipitation method of producing molding powders. The present process eliminates a quality control problem, enhances reliability in regard to those features which are affected by homogeneity, and eliminates a potential safety hazard caused by free oxidizer.

This process contrasts with the old, but frequently used process for compounding propellant powders

15 which involves preparing a solution of the soluble binder material, suspending the solid components in the solution, and precipitating the binder by quenching with a nonsolvent. The agglomerated mixture of ingredients is separated from the supernatant liquids, and 20 then dried, and sometimes screened. Although this is often called a coating process, it is in fact a simple agglomeration with solid particles randomly and mechanically held in a matrix of binder material. Often by this process, old in the art, ammonium perchlorate, the 25 most widely used oxidizer, dissolves or recrystallizes in polar solvents which contain water resulting in changes in oxidizer particle size distribution in the final product.

In the present invention with the rubber based propellant formulations Teflon is used as a reinforcing agent. Teflon will, during a shearing procedure, coalesce and cold draw into fibers. Thus, with the Teflon powder-rubber mixture, the conventional extrusion procedure results in the formation of reinforcing fibers in situ. All the fibers are never really completely 30 straight, for there is a certain amount of sideways drift of particles during extrusion. Teflon content as low as  $\frac{1}{2}\%$  effectively improves the tensile strength and % elongation of propellants containing it. The strength increases as the Teflon content is increased.

35 Several hundred measurements have been made on 0.125-inch diameter strands of the extruded mixed-binder (i.e., Teflon/rubber) propellants. The tensile strengths were generally in the range 300 to 800 psi and the percent elongations in the range of 20 to 35%.

In general the burning rates of these propellants measured with 0.125-inch diameter strands are about 0.5 in/sec at 1000 psi and ambient temperature. Slopes vary from 0.45 to 0.70 with butyl rubber, and from 0.6 to 0.8 with ethylene propylene rubber.

The following examples in Table I below present motor firing data for the mixed binder extruded propellants formulated as follows:

TABLE I

| Ex. | Propellant Formulation<br>Ingredients Wt. %                   | Theoretical            |                               | Measured               |                               | Efficiency<br>% |
|-----|---------------------------------------------------------------|------------------------|-------------------------------|------------------------|-------------------------------|-----------------|
|     |                                                               | I <sub>sp</sub><br>sec | Density<br>lb/in <sup>3</sup> | I <sub>sp</sub><br>sec | Density<br>lb/in <sup>3</sup> |                 |
| 1   | Butyl rubber<br>Teflon<br>Ammonium<br>perchlorate<br>Aluminum | 8<br>2<br>70<br>20     | 264.3<br>0.068                | 237.0<br>0.067         |                               | 89.6            |
| 2   | Butyl rubber<br>Teflon<br>Ammonium<br>perchlorate<br>Aluminum | 9<br>3<br>68<br>20     | 264.0<br>0.068                | 232.0<br>0.066         |                               | 87.9            |
| 3   | Butyl rubber<br>Teflon<br>Ammonium<br>perchlorate<br>Aluminum | 6<br>7<br>70<br>17     | 260.5<br>0.070                | 233.0<br>0.068         |                               | 89.4            |

TABLE I - Continued

| Ex. | Propellant Formulation<br>Ingredients Wt. %            | Theoretical     |                               | Measured        |                               |
|-----|--------------------------------------------------------|-----------------|-------------------------------|-----------------|-------------------------------|
|     |                                                        | $I_{sp}$<br>sec | Density<br>lb/in <sup>3</sup> | $I_{sp}$<br>sec | Density<br>lb/in <sup>3</sup> |
| 4   | Butyl rubber 7<br>Teflon 16<br>Ammonium perchlorate 77 | 242.0           | 0.066                         | 227.0           | 0.065 93.8                    |

Strand burning rates at 77° F. and 1,000 psi of three of the present new formulations are given below:

TABLE II

| Propellant Composition<br>(% by weight) |        |      |      | Rate<br>(in/sec) | Slope<br>$\Delta$ rate/<br>$\Delta$ pressure |
|-----------------------------------------|--------|------|------|------------------|----------------------------------------------|
| Butyl                                   | Teflon | Al   | AP   |                  |                                              |
| 8.0                                     | .0     | 19.0 | 70.0 | 0.48             | 0.49                                         |
| Ethylene-propylene                      |        |      |      |                  |                                              |
| 10.0                                    | .0     | 17.5 | 72.5 | 0.50             | 0.81                                         |
| 8.5                                     | 3.5    | 16.0 | 72.0 | 0.41             | 0.87                                         |

In Table III hereinbelow the theoretical performance is given of a number of propellants prepared as herein disclosed:

TABLE III

| THEORETICAL PERFORMANCE OF NEW PROPELLANTS |        |    |    |            |        |               |                      |
|--------------------------------------------|--------|----|----|------------|--------|---------------|----------------------|
| Composition, %                             |        |    |    | Ballistics |        |               |                      |
| Butyl                                      | Teflon | Al | AP | $I_{sp}$   | $\rho$ | $\rho I_{sp}$ | Chamber<br>Temp., °F |
| 12                                         | 0      | 0  | 88 | 248        | 1.72   | 427           | 4,813                |
| 12                                         | 0      | 2  | 86 | 251        | 1.73   | 433           | 4,928                |
| 12                                         | 0      | 8  | 80 | 258        | 1.75   | 452           | 5,269                |
| 12                                         | 0      | 10 | 78 | 260        | 1.76   | 458           | 5,376                |
| 12                                         | 5      | 10 | 73 | 256        | 1.77   | 454           | 5,197                |
| 10                                         | 0      | 0  | 90 | 252        | 1.75   | 442           | 4,968                |
| 10                                         | 5      | 2  | 83 | 251        | 1.77   | 444           | 5,026                |
| 10                                         | 5      | 4  | 81 | 253        | 1.78   | 450           | 5,150                |
| 10                                         | 0      | 6  | 84 | 258        | 1.78   | 460           | 5,381                |
| 10                                         | 5      | 6  | 79 | 255        | 1.79   | 456           | 5,268                |
| 10                                         | 5      | 10 | 75 | 259        | 1.80   | 467           | 5,490                |
| 10                                         | 3      | 15 | 72 | 263        | 1.83   | 480           | 5,796                |
| 10                                         | 3      | 17 | 70 | 264        | 1.84   | 484           | 5,880                |
| 9                                          | 3      | 15 | 73 | 263        | 1.85   | 485           | 5,915                |
| 9                                          | 4      | 17 | 70 | 263        | 1.86   | 488           | 5,975                |
| 9                                          | 3      | 19 | 69 | 264        | 1.87   | 493           | 6,084                |
| 9                                          | 4      | 20 | 67 | 264        | 1.87   | 494           | 6,079                |
| 8                                          | 15     | 0  | 77 | 243        | 1.82   | 441           | 4,857                |
| 8                                          | 5      | 2  | 85 | 253        | 1.81   | 457           | 5,097                |
| 8                                          | 10     | 2  | 80 | 250        | 1.82   | 454           | 5,072                |
| 8                                          | 5      | 4  | 83 | 255        | 1.82   | 463           | 5,270                |
| 8                                          | 5      | 6  | 81 | 257        | 1.83   | 469           | 5,422                |
| 8                                          | 4      | 15 | 73 | 262        | 1.87   | 489           | 5,992                |
| 8                                          | 4      | 17 | 71 | 263        | 1.88   | 493           | 6,088                |
| 8                                          | 3      | 17 | 72 | 263        | 1.88   | 493           | 6,113                |
| 8                                          | 3      | 19 | 70 | 264        | 1.89   | 497           | 6,202                |
| 8                                          | 2      | 20 | 70 | 264        | 1.89   | 499           | 6,271                |
| 8                                          | 4      | 20 | 68 | 264        | 1.89   | 499           | 6,208                |
| 7                                          | 5      | 15 | 73 | 261        | 1.90   | 497           | 6,055                |
| 7                                          | 6      | 17 | 70 | 261        | 1.90   | 497           | 6,137                |
| 7                                          | 15     | 19 | 59 | 257        | 1.93   | 496           | 5,888                |
| 6                                          | 15     | 2  | 77 | 248        | 1.86   | 462           | 5,033                |
| 6                                          | 10     | 6  | 78 | 254        | 1.87   | 476           | 5,405                |
| 6                                          | 7      | 17 | 70 | 261        | 1.93   | 501           | 6,201                |
| 5                                          | 7      | 17 | 71 | 259        | 1.95   | 505           | 6,262                |

Burning rate modifiers were incorporated into the formulations and strand burning rate results were made at 77° F. and 1,000 psi. Up to 3% modifier selected from the group consisting of cuprous oxide, cupric ox-

ide, copper chromate and ferric oxide were used. The following is a typical example:

| Ingredients          | Percent by weight |
|----------------------|-------------------|
| Butyl rubber         | 8                 |
| Teflon               | 3                 |
| Aluminum             | 19                |
| Ammonium perchlorate | 70                |
| Copper chromate      | 3                 |

20 Butyl rubber was mixed into the solvent, petroleum ether, to which Teflon, aluminum and ammonium perchlorate crystals (in a ratio of 1:1 as received, 190 $\mu$  average diameter, and ground 8 $\mu$  average diameter) were blended to form a paste. The paste was extruded into 25 burning rate strands from which the following data was derived: burning rate, 0.98 in/sec, slope  $\Delta$  rate/ $\Delta$  pressure 0.53.

30 Butyl rubber used herein is a synthetic rubber produced by polymerizing isobutylene or alternatively by copolymerization of isobutylene (approximately 98%) with a small proportion (2%) of conjugated diene, for instance isoprene or butadiene, and is identified more specifically as isobutylene-isoprene rubber (IIR). The ethylene-propylene rubber (EPR) is an elastomer made 35 by the steriospecific copolymerization of ethylene and propylene and alternatively a small percent, 2 - 5%, of a conjugated diene is added to provide curing sites.

What is claimed is:

1. A propellant molding powder comprising: from about 70 to 90 percent by weight inorganic oxidizer; up to about 20 percent by weight polytetrafluoroethylene; and from about 5 to about 15 percent by weight of a synthetic rubber selected from the group consisting of butyl rubber, ethylene propylene rubber and mixtures thereof.
2. The powder in accordance with claim 1 wherein the oxidizer is ammonium perchlorate.
3. The powder in accordance with claim 1 containing additionally up to about 20 percent by weight metallic fuel.
4. The powder in accordance with claim 3 containing additionally up to about 3 percent burning rate modifier.
5. The powder in accordance with claim 3 wherein the fuel is aluminum.
6. The powder in accordance with claim 5 wherein the oxidizer is ammonium perchlorate.
7. The powder in accordance with claim 4 wherein the oxidizer is ammonium perchlorate, the fuel is aluminum and the burning rate modifier is copper chromate.

\* \* \* \* \*